

# UNITED STATES PATENT OFFICE.

WILLIAM FRANCIS FOX, OF WHITESTONE, NEW YORK, ASSIGNOR, BY MESNE ASSIGNMENTS, TO NATURAL COLOR PICTURES COMPANY, INC., OF NEW YORK, N. Y., A CORPORATION OF NEW YORK.

## PRODUCTION OF COLORED PICTURES.

1,256,675.

Specification of Letters Patent. Patented Feb. 19, 1918.

No Drawing.

Application filed January 13, 1917. Serial No. 142,245.

To all whom it may concern:

Be it known that I, WILLIAM FRANCIS Fox, a subject of the King of Great Britain, residing at Whitestone, in the county of 5 Queens, city and State of New York, have invented certain new and useful Improvements in Production of Colored Pictures, of which the following is a specification.

My invention relates to a photographic 10 process for the production of colored pictures and while applicable to the production of single photographs in color it is peculiarly adapted for use in connection with the production of colored photographs in continuous 15 series for use in the art of cinematography.

My present invention is in some respects 20 an improvement upon that of my Patent No. 1,166,123 dated December 28, 1915, entitled Photographic process, and in other respects 25 it may be considered as providing certain steps alternative to those described in my said patent. In the patent referred to, the steps, generally speaking, may be described 30 as follows:

Two negative images are first produced, one taken through a red filter and the other through a green filter, or in more general 35 language, I produce two negative images of an object from one of which certain color sensations have been omitted and from the other of which certain other complementary color sensations have been omitted. The first mentioned image, namely, that taken 40 through the red filter is imprinted upon transparent or translucent sensitized material and colored with a color corresponding to the sensations omitted from the corresponding negative, that is to say, bluish green. The second image is then imprinted upon the material in registry with the first 45 image and colored to a color corresponding to the sensations omitted from the corresponding negative, namely, red. In the process described in my said patent, the first 50 image is given its bluish green color by toning the same by a suitable toning bath containing ferric salts, potassium ferricyanid and hydrochloric acid. The development of the second image serves to decolor the first image and the color of this first or bluish green image is restored by treating the sen-

sitized material in a bath which simultaneously restores the color to the first image and mordants the second image. The bath 55 used for this purpose in my said patent is a solution of vanadium chlorid in oxalic acid with potassium ferricyanid. The second image is then dyed with a basic red dye 60 which combines with the color imparted by the mordant mentioned, to give the desired red to the second image.

In accordance with my present invention the above method of procedure is followed with differences which will now be pointed 65 out. The first print, viz., that made from the red negative, is developed and instead of being toned to a blue color in a bath containing potassium ferricyanid and ferric salts, it is treated with one bath containing 70 potassium ferricyanid and after washing, is immersed in another bath containing the necessary ferric salts. The first bath mentioned may contain potassium ferricyanid, water and ammonia which bleaches the black 75 silver image to white. The second bath may contain ferric ammonium oxalate, water and hydrochloric acid which colors the print to the desired blue. This differs from the process described in my patent referred to in that 80 the potassium ferricyanid and the ferric salts are in separate baths. This is an improved proceeding because thereby I avoid precipitation which takes place when the ferric salts and potassium ferricyanid are 85 mixed together.

The second point of improvement consists in the following: After the second print has been made it is developed and immersed in the same bleaching bath as was used for the 90 blue image. It is then washed and immersed in a bath containing uranium nitrate with water and hydrochloric acid. The immersion in the bleaching bath converts the black silver deposit on the sensitized material to 95 silver ferrocyanid which reacts with the uranium contained in the second bath to form uranyl ferro-cyanid which is an orange-red color complementary to the blue of the first image. By this procedure I am 100 enabled to obtain excellent results with less operations and in less time than in the procedure described in my patent referred to in which vanadium salts and a basic dye were

used for obtaining the red color. It is sometimes found advisable to mix a solution of some basic red or other color dye with the uranium solution, the uranium acting as a 5 mordant for the red dye as it is precipitated in the film. This is not absolutely necessary but the addition of the basic red dye makes the red color produced a more vivid crimson than in the case in which the uranium solution 10 is used without the basic dye. Likewise, basic orange or yellow dyes may be used to give a more vivid orange or yellow red.

By this method I am enabled to color 15 prints a very desirable red and this step of my process is of wide applicability. Uranium toning has been previously proposed but has not been of practical value, so far as I am aware, because of the uncertain results 20 that were attained. It may be stated briefly that uranium is a radio-active material and is affected by light, so that consistent results with the same have been difficult of attainment. In the method described herein, however, 25 in which the potassium ferricyanid and the uranium salts are used in separate baths and the procedure and proportions herein-after more fully described are employed, excellent and uniform results are obtained.

30 The details of the procedure described may now be given somewhat more fully.

The first step in the process comprises producing a suitable negative. A series of pictures is taken by means of a camera employing a red and green colored filter, the images being taken alternately through the red and green portions of the filter. This negative is made upon suitable transparent or translucent material; such, for example, as py- 35 roxylene stock coated with silver bromid emulsion and extra sensitized to be panchromatic. The negative strip is then developed, fixed, washed and dried in well known manner.

40 A positive is then made, the first step consisting in reproducing in straight line sequence all of the images taken through the red filter. The print thus made is upon transparent or translucent film-stock coated with silver bromid emulsion, not necessarily 45 panchromatic, the sensitized emulsion preferably being upon but one side of the stock. After the development of this print from the red negative the same may either be 50 fixed or left unfixed, as good results may be obtained by either method. It is then placed in a bath consisting of potassium ferricyanid and ammonia in approximately the following proportions:

60 Potassium ferricyanid 1 lb.  
Water 10 lbs.  
Ammonia (.880) 8 ounces.

This will bleach the black silver image to 65 a white, which takes from three to five min-

utes. It is then washed to remove the bleacher, and immersed in another bath containing

Ferric ammonium oxa-  
late 1 lb.  
Water 10 lbs.  
Hydrochloric acid 4 ounces.

70

The image is then fixed in a sodium thiosulfate solution, is again washed, dried and 75 is ready for the application of the second print. This has toned the image a rich transparent blue color.

The positive strip may now be given a second coating of emulsion, the operation 80 being performed at such a temperature that the second coating will in practical effect combine with the first coating to make essentially but a single homogeneous coating upon the underlying film stock. I may also 85 proceed, if desired, without recoating the stock. Assuming that the film is re-coated, the next step consists in impressing upon the positive strip and in precise superposition upon the image already there, the 90 image of the green negative, that is, the negative taken through the green filter. After this green image has been printed upon the positive, the positive strip is developed and is either fixed or left unfixed, as desired. The positive strip is then immersed 95 in the same bleaching bath as was used for the blue image, namely, the bath consisting of potassium ferricyanid and ammonia and when the action is complete is washed to 100 remove traces of the bleaching bath. The strip is then immersed in the uranium bath of which the following is the best example.

Uranium nitrate 8 oz.  
Water 10 lbs.  
Hydrochloric acid 4 ounces.

105

The strip is left in this bath for approximately five minutes, after which it is fixed, and washed for half an hour when it is 110 ready for drying and projecting in a moving picture projecting machine.

The development of the second image results in a bleaching-out and entire obliteration of the bluish green color from the first 115 image, although the image itself remains faintly visible. This is the same effect as noted in my patent referred to above, and this effect ensues because the first image impressed upon the positive film is open to 120 the action of any solution which may be used in the treatment of the second image, no attempt being made to protect the same. This color is restored to the first image, by the acid in the uranium nitrate and hydro- 125 chloric acid bath, this bath being sufficiently acid to restore the color to the first image. The immersion of the film in the potassium ferricyanid bath after the second print has been developed, converts the black silver de- 130

5 positi of the second print to silver ferrocyanid and the reaction in the second bath with the uranium contained therein forms a substance which is apparently uranyl ferro-cyanid, and which is an orange red color complementary to the blue of the first image.

10 In many cases it is advisable to mix a solution of some basic red dye with the uranium nitrate solution, the uranium acting as a mordant for the red dye as it is precipitated in the film. A strength of dye of about .001 per cent. is employed and the dye used may be of any of the basic dyes mentioned in my patent above referred to or other suitable basic dyes. The dye may be used as stated when it is deemed advisable to have a red of a more vivid color than is produced by the uranium bath without the basic dye.

15 As stated, the second print may be superposed upon the first without first re-coating the film in the same manner as is described in my patent above referred to. If but a single coating of emulsion on the positive film stock is to be employed, the film, after the development of the first printing should be immersed in a combined washing bath containing, however, a small percentage such as one per cent. of acetic acid, this operation being carried out in the dark room and being intended to wash out surplus developing solution and to arrest the process of development. When the first image is printed upon the positive strip, in this case care should be taken that the exposure be not so great as to affect the entire mass of the sensitive coating. Therefore the first image will in effect be portrayed in the upper layer of the coating, the emulsion underlying it remaining sensitive and it is this sensitive portion of the emulsion which is utilized in impressing the second print upon the positive strip, this operation not being interfered with by the image already there, which has been turned a bluish green and therefore obstructs the passage of light but little, if at all.

20 It should be particularly noted that I am enabled by the processes outlined, to obtain results with the uranium toning operation which are uniformly excellent, such results being obtained, however, only as a result of a long period of experimentation. If a basic red dye is additionally used, suitable dyes will include rhodamin azin red, acridin red and saffranin red. If a vivid shade of red different from crimson is desired, other suitable dyes, such as basic orange or basic yellow dyes, may be used.

25 Having now described my invention, what I claim and desire to secure by Letters Patent is:—

1. A photographic process comprising, imprinting a negative image of an object,

from which certain color sensations have been omitted, upon light-transmissive sensitized material, coloring said image bluish green, imprinting a second image of the same object, from which other color sensations have been omitted, upon said material in registry with the first image imprinted thereon, developing said second image, immersing the material in a bleaching bath containing potassium ferricyanid, washing, and immersing in a bath containing uranium nitrate and hydrochloric acid and fixing and washing the second image, substantially as described. 70

2. A photographic process comprising, imprinting a negative image of an object, from which certain color sensations have been omitted, upon light-transmissive sensitized material, developing, bleaching the print in a bath containing potassium ferricyanid and ammonia, washing, toning the print in a bath containing ferric-ammonium oxalate and hydrochloric acid, fixing, washing, imprinting a second image of the same object, from which other color sensations have been omitted, upon said material in registry with the first image imprinted thereon, developing said second image and thereby decoloring said first image; and simultaneously restoring color to said first image and coloring said second image red, substantially as described. 85

3. A photographic process comprising, imprinting a negative image of an object, from which certain color sensations have been omitted, upon light-transmissive sensitized material, developing, bleaching the print in a bath consisting of potassium ferricyanid and ammonia, washing, toning the print in a bath containing ferric ammonium oxalate and hydrochloric acid, fixing, washing, imprinting a second image of the same object, from which other color sensations have been omitted, upon said material in registry with the first image imprinted thereon, developing said second image, immersing the material in a bleaching bath similar to that used for the first print, washing, immersing in a bath containing hydrochloric acid and a uranium salt adapted to form uranium chlorid with the acid, and fixing the second image, substantially as described. 100

4. A photographic process comprising, imprinting a negative image of an object, from which certain color sensations have been omitted, upon light-transmissive sensitized material, developing, bleaching the print in a bath consisting of potassium ferricyanid and ammonia, washing, toning the print in a bath containing ferric ammonium oxalate and hydrochloric acid, fixing, washing, imprinting a second image of the same object, from which other color sensations have been omitted, upon said material in 115

registry with the first image imprinted thereon, developing said second image, and coloring said second image red by means of potassium ferricyanid and a uranium salt in solution, substantially as described.

5. A photographic process comprising, imprinting a negative image of an object, from which certain color sensations have been omitted, upon light-transmissive sensitized material, coloring said image bluish-green, imprinting a second image of the same object, from which other color sensations have been omitted, upon said material in registry with the first image imprinted

thereon, developing said second image, immersing the material in a bleaching bath containing potassium ferricyanid, washing, and immersing in a bath containing uranium nitrate, hydrochloric acid and a basic dye, fixing and washing, substantially as described. 15 20

This specification signed and witnessed this 9th day of January, 1917.

WILLIAM FRANCIS FOX.

Witnesses:

DRYER SMITH,  
I. MCINTOSH.